

Jan. 31, 1933.

O. S. PETERS

1,895,519

METHOD OF PREPARING CARBON RESISTANCE STACKS

Filed June 6, 1929

Fig. 1.



Fig. 2.



Fig. 3.



INVENTOR:

Orville S. Peters,

by *Murray G. Boyer*  
Atty.

## UNITED STATES PATENT OFFICE

ORVILLE S. PETERS, OF CHEVY CHASE, MARYLAND

## METHOD OF PREPARING CARBON RESISTANCE STACKS

Application filed June 6, 1928. Serial No. 368,885.

My invention relates to the preparation of carbon stacks employed as resistance elements in various forms of electrical apparatus, measuring instruments, electric telemetric devices, etc., one instance of a structure of the latter type being illustrated and claimed in my Patent No. 1,528,627, March 3, 1925.

The object of my invention is to standardize the piles or stacks of carbon disks employed with instruments of this character whereby the pressure resistance characteristics of each of a plurality of stacks arranged in series or in multiple shall be identical and constantly reproducible so that like changes of pressure shall produce like changes of resistance in the several stacks.

In the construction and development of electric telemetric measuring instruments of the type disclosed in my patent above referred to, employing a pair of carbon stacks arranged in series, it is essential that the pressure resistance characteristics of these stacks shall be identical and constantly reproducible.

The deflections of an instrument such as indicated at 32 in my patent above referred to depend upon the current, indicated by the ammeter associated therewith which in turn indicates the changes of resistance in the carbon stacks arranged in series. In order that these deflections may be alike from time to time under like conditions of measurement, it is necessary that the changes of resistance of each of the carbon stacks be the same for like conditions, and in order that I may produce stacks fulfilling these requirements, I have developed an improved method of preparing the carbon rings or disks and of forming the stacks.

In the employment of pairs of carbon stacks in the relation indicated in my patent above referred to, it is essential that each stack possess the same pressure resistance characteristics. For instruments using single stacks it is also important that each stack possess the same pressure resistance curve, because in cases where single stacks are built into separate instruments the similarity of the stacks reduces the labor otherwise necessary to adjust the several instruments to give like readings under like conditions.

In the commercial production of carbon stacks it has proved difficult to coordinate stacks of carbon disks made in different batches and to insure that the pressure resistance characteristics of one group of carbon disks arranged in a stack will be identical with the pressure resistance characteristics of another stack having the same number of carbon disks. I have discovered that, in order to produce stacks having identical pressure resistance characteristics, not only must the stacks contain the same number of disks but if the stacks having the same number of disks can be made to have the same resistance under one pressure, similar variations in pressure will produce similar resistances in the different stacks and the parabolas indicating their pressure resistance changes will be identical. The object of my invention is to reproduce in pairs, or other convenient quantities, stacks or piles of carbon disks each having the same number of disks and in which the pressure resistance characteristics will be the same and constantly reproducible.

In the accompanying drawing I have indicated diagrammatically carbon rings or disks made in accordance with my invention, in which:

Figure 1 indicates a pile of carbon disks; Fig. 2 an enlarged plan view of a single disk, and

Fig. 3 an elevation of Fig. 2.

The carbon rings or disks indicated at 10 are usually mounted in stack form; Fig. 1, illustrating a vertical stack, and disposed between metal members 11 to which conducting wires 12 may be connected; such members 11 being separated from metal plates 13 forming part of supporting means for the carbon stacks, by insulating disks 14.

These carbon rings or disks in completely finished form are approximately .018 to .02 inches in thickness, and the piles or stacks employed as pressure resistance elements may comprise fifty (50) of these rings or disks.

The carbon disks making up the stacks em-

- ployed in devices of the character set forth in my patent referred to may be produced from various materials such, for example, as powdered coke, graphite, etc., which may be carbonized under heat and pressure and in practice I have used a number of easily available materials, the particulars of which it seems unnecessary to note. In preparing the disks employed in these carbon stacks, I find that the resistance of the disks of successive batches will vary in relatively wide ranges and with a view of preparing stacks having a known resistance of a suitable quantity, I may proceed as follows.
- 15 The material employed in the manufacture of these carbon disks is initially granular or pulverulent, and is compressed into substantially the final form by suitable means. To insure that the respective disks shall have the same amount of material, compressed to the same degree, and of the same thickness, such compressing means are preferably arranged so that excess material may flow through apertures of the dies to insure that 20 the salient features mentioned can be uniform, insofar as the preliminary steps are concerned, in the production of successive rings or disks of such material subsequently carbonized.
- 25 30 In the use of the material from which these carbon disks are produced, a binder may be employed and the first step after compression is a baking operation which sets such binder (when used) and insures coherence of the compressed particles of the material employed in the subsequent heat treatment. This baking operation may be carried on at a temperature of about  $130^{\circ}$  C. for a period of approximately three hours.
- 35 40 From the baking chamber the rings or disks are introduced into a carbonizing furnace and are slowly brought to a red heat at a temperature of about  $650^{\circ}$  C., within a period of approximately forty-eight hours.
- 45 50 55 The heat is then shut off and the carbon rings or disks are allowed to cool slowly in the container in which they have been carbonized. During the carbonizing treatment, the disks are embedded in lamp black for the purpose of consuming any oxygen in the material employed or in the chamber in which carbonization takes place, and to insure a complete exclusion of air, the chamber or container receiving the disks for carbonization is embedded in a body of lime or similar material.
- This method of manufacture produces batches of these carbon disks at each operation, and the usual practice is to carbonize the same quantity at each operation. In my practice I have carbonized batches of one thousand disks. Following carbonization, the disks are ground on opposite faces to insure uniformity of the surface and that such faces shall be parallel and flat.

I have found, despite all precaution that may be taken in connection with the character of the pulverulent material employed; the fineness of the particles or granules thereof; the character of the binder (when used); the pressure effected during the formation of the rings or disks; the baking treatment; the carbonizing treatment, and finally the grinding operation, that the annular disks do not possess identical pressure resistance characteristics.

In the development of the carbon stacks as I have carried the same into effect, it has been desirable, for instance, to produce stacks, say of 50 discs whose total resistance 80 may be approximately eighty (80) ohms at a total pressure of twenty (20) pounds. I have found that the resistance of the respective stacks of carbon disks at this pressure may vary between 50 and 150 ohms.

For example, although it is possible to produce a batch of disks, fifty (50) of which will give a resistance of 1200 to 1350 ohms; another batch of which any fifty (50) disks will give a resistance of between 1400 and 90 1450 ohms and so on, it is impossible to produce a batch from which two stacks of fifty (50) disks may be picked at random which will give the same total resistance at the same pressure, say 1220 ohms.

It has heretofore been the practice to increase or decrease the number of disks in the stack to make the resistances of two stacks under given pressure the same. The result of the practice of this method was to 100 produce stacks in no two of which a change in pressure would produce identical changes in resistance, i. e., in no two of which would the pressure resistance parabolas be identical.

In order to utilize my discovery and produce standardized stacks in each of which the resistance will be equal at all of a plurality of pressures, I have found that by carefully assorting disks from respective batches I can develop standardized stacks 110 containing equal number of discs, all stacks possessing identical and constantly reproducible pressure resistance characteristics.

The basis for this method of producing standardized stacks from different batches 115 having different pressure resistance characteristics is found in the fact that the pressure resistance characteristic of a plurality of carbon disks is a parabola of the form

$$x^2 = 2p(y + h),$$

where "x" relates to pressure, "y" to resistance, and "p" and "h" are constants.

I have found experimentally that for carbon stacks of the same material, but having 125 unlike resistances for the same pressure, the pressure resistance curve can be made to fit the curve of the equation above referred to by plotting to the proper scale, within the limits of experimental errors. Thus it ap- 130

pears that the individual pressure resistance characteristics of a plurality of stacks of the same material, but prepared at random, form a family of curves.

5 The process of standardizing the stacks then consists in selecting some particular curve, for instance, one in which a standard stack shows 80 ohms at 20 pounds total pressure, and selecting disks from batches having greater and less resistance at this pressure in sufficient number and ratio so that when stacked up the average resistance at the given pressure shall be the required value. In practice, this operation is readily 10 15 20 25 30 35 40 45 50 55 60 65 70 75 80 85 90 95 100 105 110 115 120 125 130

A stack so prepared, being composed of elements having the same fundamental characteristics in different degree, presents an average characteristic which can be repeated in an indefinite number of stacks if the elements are properly selected, although it is not necessary that the elements be the same in every case. It is necessary only that the average be the same in every case.

For example, after preparing the first stack so as to obtain the desired resistance at a given pressure, an indefinite number of stacks may be prepared, each having the same resistance as the first stack at all pressures, by having the same number of disks in each stack as is in the original stack and substituting disks of different resistances until at any one pressure common to both the original stack and the stack being formed the resistance is the same and, this result being attained, the resistances of the stacks will be the same at all pressures.

Thus the preparation of stacks of disks as regards standardization of their pressure resistance characteristics is removed from the chance of random selection and placed upon a physico-mathematical basis which permits the formation of large numbers of stacks to exact specifications.

I claim:

1. The method of forming a plurality of resistance stacks, which comprises forming one stack having the desired resistance characteristics of a plurality of carbon discs of non-uniform resistance characteristics, and forming succeeding stacks of the same number of discs as the first stack but selecting the discs so that the total resistance of each succeeding stack is the same as that of the first stack at any common pressure.

2. The method of forming a plurality of resistance stacks having identical pressure resistance parabolas, which comprises selecting and assembling a plurality of resistance discs having non-uniform resistance

characteristics in sufficient number to give the desired total resistance of the stack at a given pressure and forming subsequent stacks by assembling the same number of discs into stacks but selecting said discs to impose the same resistance as is imposed by the first stack at any common pressure.

3. The method of forming resistance stacks composed of a plurality of disks having non-uniform pressure resistance characteristics, which comprises selecting and assembling sufficient disks to produce a stack having the pressure resistance characteristics desired, and forming each subsequent stack of the same number of disks as is contained in the first stack but selecting the disks so that the sum of the resistances is equal to the resistance offered by the first stack under a similar pressure, whereby the resistance offered by said subsequent stacks will be the same as that of the first stack at every common pressure.

4. The method of forming a plurality of resistance stacks having a common pressure resistance parabola from disks having non-uniform pressure resistance characteristics, which comprises selecting and assembling a plurality of disks to form a stack having the desired resistance at a given pressure; forming all subsequent stacks by assembling the same number of disks as in the first stack; and varying the resistivity of the stack to approach the desired form by substituting disks of greater or lesser resistances while maintaining constant the number of disks in the stack.

In witness whereof I have signed this specification.

ORVILLE S. PETERS.

105

110

115

120

125

130